

## UNITED STATES PATENT OFFICE

2,339,520

## RECLAIMING LUBRICANTS

August H. Riesmeyer, Arnold, Pa., assignor to  
 Aluminum Company of America, Pittsburgh,  
 Pa., a corporation of Pennsylvania

No Drawing. Application June 27, 1940,  
 Serial No. 342,695

4 Claims. (Cl. 196—16)

This invention relates to the reclamation of metal working lubricants, and particularly to the reclamation of lubricants used in the working of light metals, aluminum and magnesium, by the removal of contaminating substances to make the lubricants suitable for further use in metal working processes.

While lubricants are used in many types of cold working processes in the fabrication of aluminum and magnesium products, they are used most extensively in rolling aluminum and magnesium sheet, strip, and foil products, and for this reason the present invention is described in connection with the reclamation of lubricants used in the rolling process, though it is apparent that the invention can be advantageously employed in the reclamation of lubricants used in other fabrication processes employed with these materials.

The lubricants used in the rolling of light metals perform several functions. They appear to help the passage of the metal through the rolls, permitting relatively high gauge reductions in the individual roll passes. They also perform the function of reducing the heat generated in the rolling process both by reducing the friction and by their action as a coolant. Obviously, to obtain any appreciable cooling, the lubricants must be supplied in rather large quantities. Another important function of these lubricants is the protection which they afford the metal against marring and scratching when the metal is stacked or coiled subsequent to the rolling operation.

The principal lubricants which have been used in the rolling of light metals are well refined mineral oils varying from 45 seconds to 1000 seconds Universal Saybolt viscosity. Lubricants of this character can be used alone, but generally they are provided with from 1 to 20 per cent of various modifying agents. Specifically, these modifying agents are usually selected from the group consisting of the fixed oils or fats such as palm oil, cocoanut oil, cotton seed oil, peanut oil, sperm oil, fish oil, spermaceti, tallow, lard fat, and horse fat, or mixtures of these materials.

The mills used in the rolling of light metals are usually provided with circulating systems to feed the lubricants to the entry side of the rolls, and the systems are adapted to recirculate the excess oil. After a relatively short period of use, the lubricants become contaminated and rendered unfit for further use, though their lubricating properties are not noticeably impaired.

The conditions under which such lubricants are used give rise to several contaminating influences which make the lubricant unsuitable for

further use. Probably the principal contaminating substances in oil which has been used in these processes are the oxidation products of the oil itself, solid carbonaceous matter formed by the 5 partial decomposition of the oil, particles of the metal being worked, and oxidation products of the metal being worked.

It has been found economically unfeasible to reclaim these contaminated lubricants by means 10 of any of the presently known mechanical separation processes, such as sedimentation and decantation, filtering, or centrifuging. This difficulty probably arises from the fact that many of the contaminating substances present are extremely fine, being substantially colloidal in 15 nature, and apparently will pass through even the finest filtering media which can be practically used. The larger particles can be removed by various mechanical separating processes, but 20 the removal of these larger particles does not render the lubricant fit for reuse in fabrication processes. Among the principal contaminating substances which are not removed by the usual mechanical separating processes appear to be extremely finely divided particles of the metal or 25 of the oxide of the metal, together with finely divided carbonaceous matter.

These contaminating substances, despite their 30 extremely finely divided form, cause defects in the finish of light metal products which render the products commercially unacceptable. The larger of the particles, probably finely divided metal or oxide of the metal being worked, cause marking or marring of the surface and frequently, in the case of rolling thin metal foil, actually result in perforation of the material produced. Another defect caused in light metal products is the staining of the product during heat treatment 35 due to the burning onto the surface of the solid residue of the contaminated lubricant. Stains formed in this manner are practically impossible to remove and render the material in which they appear commercially unacceptable.

The present invention is predicated upon the 40 discovery that these contaminating substances can be removed from the lubricant by treating the lubricant with certain reagents which will either combine with the metal or the oxide of the metal being worked in the fabrication process, forming salts or compounds which can be subsequently readily removed from the lubricant, or which, when present in the lubricant, do not impair its characteristics and render it satisfactory for reuse in metal fabrication processes. 45 The amounts of these reagents used may be com-

puted in terms of the metallic content of the contaminated lubricant, and when so employed, these reagents appear to dissolve or otherwise to make it possible to remove all of those contaminating substances present in the lubricant that make it unfit for further use in metal working processes.

The specific reagents which have been found to effect a satisfactory reclamation of these contaminated lubricants are sulphuric and hydrochloric acids. That these reagents could be satisfactorily used in the reclamation of such lubricants is directly contrary to the opinion generally held in the metal working arts where it has been believed that the contact of refined lubricants with strong mineral acids should be avoided under all circumstances. The presence in a lubricant of strong mineral acids, even in relatively minute amounts, leads to the rapid deterioration of the equipment with which it is used, particularly with finely finished equipment such as the rolls used in the rolling of light metal products. It has been discovered that sulphuric acid and hydrochloric acid can be added to these lubricants in amounts effective to remove the contaminating substances without apparently increasing the corrosive nature of the lubricants when used in light metal fabrication processes. Apparently, these reagents combine with the light metal and/or the oxide of the light metal to form compounds which can either be entirely removed by mechanical separation processes or which, if present in the lubricant, do not have any deleterious effects. Even if a slight excess of either of these reagents is used, as compared with the amount necessary to combine with all of the light metal or light metal oxide, the reuse of these lubricants in a light metal forming process brings them almost immediately in contact with the light metal being worked, thus almost immediately neutralizing any excess acidity.

In general, it has been found that sulphuric acid is the most effective reagent for removing these fine or colloidal contaminating substances present in lubricants used in the fabrication of light metals. This reagent, when added in the stoichiometric or slightly less than the stoichiometric amount necessary to combine with the metallic impurity in the lubricant, permits a complete separation of the contaminating impurities from the lubricant without in any manner impairing its suitability for reuse. Even when added in amounts slightly in excess of the amount which will combine with all of the metal present in the lubricant, the lubricant is satisfactory for reuse.

It is merely necessary that this reagent be added to the lubricant and thoroughly mixed therein and the lubricant be allowed to stand for a reasonably short period of time, and apparently all of the solid contaminating substances which would render the lubricant unfit for further use will settle out and the clarified lubricant can be decanted from a vessel in which the material has been allowed to stand. A somewhat more complete recovery of the lubricant can be obtained by extracting it from the residue remaining after the decantation operation by centrifuging or filtration.

Hydrochloric acid can be substituted as a full equivalent for the sulphuric acid, but it is not generally as satisfactory because the solids usually have to be separated from the lubricant by centrifuging or filtering rather than by sedimentation and decantation.

In the specification and claims the expression "light metal or metallic content of the lubricant" is used to define the total metal present in the lubricant in the form of free metal and the oxide 5 of the metal. It is also significant that the amount of reagent added to the lubricant in the practice of the invention is computed on the basis of the metal present in the lubricant in the form of free metal and its oxide.

10 It is generally preferable to use these reagents in as highly concentrated form as is practical at temperatures below about 65° C. as it has been found that highly concentrated acids are more effective and because the time required in the 15 settling operation following the addition of the acid may be greatly reduced. If, however, the lubricant being treated contains a large amount of fatty acid and it is desired to employ sulphuric acid as a reagent, it is usually advisable 20 to use a somewhat lower concentration of sulphuric acid. While this increases the period required to effect separation, there is less carbonization of the fatty acid with a resulting decrease in the fatty acid content of the lubricant. It 25 has been found that the time required to remove contaminating substances from the lubricant can be reduced in some instances by the addition of alcohol or a mixture of alcohol with small quantities of certain commercial detergents, and particularly those detergents consisting principally 30 of sodium salts of the sulphuric acid reaction products of aliphatic alcohols. These additions are not necessary to the successful operation of the process but they do effect a reduction in the 35 time required to obtain the separation of the solid impurities from the lubricant.

The amount of either of these acids (HCl and H<sub>2</sub>SO<sub>4</sub>) which should be added to any given contaminated lubricant may be determined by slowly adding the acid to the lubricant while subjecting it to vigorous agitation. While undergoing this treatment, the lubricant immediately starts to lose its darkened appearance, and the addition of the acid should be discontinued as soon as the 45 lubricant appears to be completely clarified. The lubricant is then allowed to stand for a period of time, preferably about 24-48 hours. During this period of standing, the compound formed, by the light metal present and the added acid, settles to the bottom of the vessel in which the lubricant has been standing. Apparently, all of the solid matter present in the lubricant settles out during this period, and the clarified lubricant can be decanted from the vessel. The decanted 50 lubricant is suitable for further use in the light metal working process without any additional treatment.

As stated before, the acid should be added in as highly concentrated form as is practical because less settling time is required. Concentrations of sulphuric acid varying from 50 to 98 per cent have been successfully used, but concentrations above 100 per cent, such as oleum (fuming sulphuric acid), are not desirable. Suitable dilution of the acid can best be obtained by using alcohol as a diluent.

A preferable method of treating the lubricant is to determine the amount of light metal present in the lubricant and then adding the acid 70 in an amount slightly less than the stoichiometric amount necessary to combine with all of the light metal present, either as the chloride of the light metal, or the sulphate of the light metal, as the case may be, depending upon the acid used. The following specific example is typical

of the treatment used with a lubricant commonly employed in the rolling of aluminum. This lubricant is specified by the suppliers as being a 45 second Pennsylvania mineral base oil having added thereto 1 per cent of horse fat and 1 per cent of sperm oil. After use for a period in an aluminum rolling process, an analysis of this oil indicated that it contained 0.028 per cent of aluminum, computed on the basis of free aluminum and its oxide. 100 gallons of this lubricant contained 0.224 pound of metallic aluminum by analysis, computed on the bases of free aluminum and its oxide. To the 100 gallon batch of the lubricant 1 pound of concentrated sulphuric acid was added. This amounted to about 85 per cent of the theoretical amount necessary to combine with the aluminum present to form aluminum sulphate. The lubricant with the acid added was agitated thoroughly for one hour at room temperature and allowed to settle for a period of 24 hours. The clarified lubricant was removed by decantation and found to be entirely suitable for reuse in the metal fabrication process in which it had been employed.

I claim:

1. The method of reclaiming lubricants consisting principally of refined mineral oils and used in the working of light metal and containing particles of the light metal being worked, which consists in treating the lubricant with sulphuric acid in an amount substantially equal to the stoichiometrical amount which will combine with all of the light metal present in the lubricant to form light metal sulphate, and subsequently separating the solid impurities from the lubricant.

2. The method of reclaiming lubricants consisting principally of refined mineral oils and used in the working of light metal and containing particles of the light metal being worked, which consists in treating the lubricant with sulphuric acid, in an amount substantially equal to the stoichiometrical amount which will combine with all of the light metal present in the lubricant, and alcohol to form a sulphate of the light metal, and subsequently separating the solid impurities from the lubricant.
- 5 3. The method of reclaiming lubricants consisting principally of refined mineral oils and used in the working of light metal and containing particles of the light metal being worked, which consists in treating the lubricant with sulphuric acid, in an amount substantially equal to the stoichiometrical amount which will combine with all of the light metal present in the lubricant, alcohol, and a sodium salt of a sulphuric acid reaction product of an aliphatic alcohol to form a sulphate of the light metal, and subsequently separating the solid impurities from the lubricant.
- 10 20 4. The method of reclaiming lubricants used in working light metals, for re-use in said working operation comprising treating a lubricant with a reagent selected from a group consisting of sulphuric acid and hydrochloric acid in an amount substantially equal to the stoichiometrical amount required to combine with all of the light metal present in the lubricant to form a salt of the light metal which is insoluble in said lubricant, and subsequently separating the solid impurities from the lubricant.
- 15 25 30 35

AUGUST H. RIESMEYER.